

Aug. 24, 1948.

**R. C. PIERCE**  
METHOD OF SIMULTANEOUSLY BEAMING  
AND ELECTROPLATING WIRES  
Filed Nov. 11, 1944

2,447,531



Inventor:  
Robert C. Pierce,  
By Clinton, Wiley, Schrader,  
Merriam, H. C. Green, A. D. Biggs.

## UNITED STATES PATENT OFFICE

2,447,531

METHOD OF SIMULTANEOUSLY BEAMING  
AND ELECTROPLATING WIRES

Robert C. Pierce, Niles, Mich., assignor to National-Standard Company, a corporation of Michigan

Application November 11, 1944; Serial No. 562,953

2 Claims. (Cl. 204—28)

1

This invention relates to a plated wire and more particularly to a beamed wire of fine diameter and low elastic limit.

Beaming comprises simultaneous winding of a plurality of wires upon a common spool. Wire is customarily beamed for numerous purposes but particularly where it is to be braided or similarly handled.

The wire which is to go on the beaming spool is customarily stored and transported on spools on which the wire is wound in a plurality of overlapping courses, each extending from one end of the spool to the other. In handling very fine wires, particularly of metal such as copper, the mere transfer from one spool to another is a matter of some difficulty and is likely to lead to considerable breakage. For example, an annealed copper wire having a diameter of 0.005 inch and having an elastic limit of 12,000 lbs. per square inch, will stretch beyond its elastic limit if the tension upon it exceeds  $\frac{1}{4}$  lb. Even with a similar wire of 0.020 inch diameter, the tension cannot exceed 4 lbs. The present invention produces a beamed product consisting of such a small wire having an electroplated coating thereon and not stretched beyond its elastic limit after or during application of the coating.

This is accomplished by mounting the take-off spools in such manner as simultaneously to feed wires at a predetermined level, passing the wires under tension below their deforming tension in a catenary path of extremely small depth to a take-up spool or drum. The wires may in their path be permitted to fall, to the extent of the depth of the catenary, into one or more baths which preferably include a cleaning bath, a pickling bath, a plating bath, and one or more washing baths. Plating is preferably by electro-deposition. It is of course impracticable to employ solid contacts within the catenary when dealing with wires of such small strength. Current is, therefore, passed through the wires by contacts which include one or more of the baths and one of the spools; preferably a power driven take-up spool or drum.

This invention is an improvement upon the developments set forth in the co-pending applications of Clare Luke, Serial No. 558,697, filed October 14, 1944, and Serial No. 560,513, filed October 26, 1944. In the present development the beaming process is combined with the Luke method of treating. Because of this combination it has been possible to eliminate a separate beaming operation which has heretofore always been required and at the same time the permissible

10 tension upon the wire was raised because of exerting this tension upon a group of wires rather than each wire separately. It should be observed, however, that the permissible tension does not increase arithmetically as the number of wires increases because of the fact that at certain stages of the process one or more of the wires may from time to time develop slack. On the whole, however, a group of very fine wires which are passed simultaneously through the baths to a common spool unite into a body having increased strength. They may even be associated in such a body through the plating bath, but for some types of plating and for some sizes of wires a small separating comb may be inserted in the plating bath to separate the wires during their passage therethrough.

20 The invention is illustrated in the drawings in which Fig. 1 is a side elevation of an apparatus suitable for practicing the invention; Fig. 2 is a plan view; Fig. 3 is an enlarged sectional side elevation showing in detail the method of suspension of the wire catenary in two of the baths; Fig. 4 is a diagrammatic enlarged view of the wire; and Fig. 5 is a transverse end elevation of a modified form of overflow.

25 The apparatus comprises a suitable mounting upon which a plurality of let-off spools 21 are mounted. A series of tensioning and spacing members 22 are provided adjacent the spool to maintain the wires 25 at substantially a predetermined vertical position. The wires pass in a body through a series of baths which will be later described to a power driven capstan 10 around 30 which the wires are wrapped several times and from which they are passed to a beaming spool 23. It will be noted that between the spacing or tensioning devices 22 and the point of contact with the capstan 10 the wires are suspended in a 35 catenary of very small depth. With 0.005 inch annealed copper wire the catenary should not be deeper than approximately  $\frac{1}{2}$  inch and is preferably about  $\frac{1}{4}$  inch. For 0.020 wire the depth of the catenary may be somewhat greater.

40 45 The series of baths comprises an alkali cleaning bath 24 preferably containing an alkali cyanide solution; a cold water rinse 3, an acid pickle bath 4, a water wash 5, a plating bath 6, a cold water wash 7, and a hot water wash 8. Each of 50 the baths is constantly supplied with fluid which overflows at the edges of the baths as shown in Figure 3. This overflow is, except in the case of the cold wash water, recycled by means of pumps 11. The surface tension of the liquid in each 55 bath forms an inverted meniscus 12 at the over-

flow 13 and the wires pass into and out of each bath through such a meniscus. In some instances the depth of the meniscus may be increased by providing narrow slots in the end of the bath through which the overflow will run and within which the wires pass. Such a slotted overflow 24 is indicated in Figure 5.

Plating current is passed through the wires as indicated in Figure 1. The electrodes 14 within the bath 2 are negatively charged. The electrodes 15 within the plating bath 6 are positively charged, and the capstan itself (or the take-up spool 23) is negatively charged. Electrons, therefore, enter the wires through the cleaning bath 2 and the capstan 10 and are withdrawn through the plating bath and the electrodes 15. Viewed in the conventional manner, current is introduced into the wires in the plating bath and passes out of them in a divided current, part to the electrodes 14, and part to the capstan 10. Conventional voltage regulators are employed to divide the current equally between these two paths.

The wires may be withdrawn from the let-off spool at a speed of 400 ft. to 500 ft. per minute. A suitable total tension is less than  $\frac{1}{4}$  lb. The cleaning bath is designed to remove saponifiable impurities and suitably is an alkali cyanide, for example one containing 2 oz. of sodium cyanide per gallon. It is preferably heated to a temperature of the order of 140° F., as, for example, by steam coils 9. Overflow liquid is recycled by the pump 11 beneath the surface of the bath, it being introduced near the bottom. An air jet 16 having a small opening immediately above the wire and directed vertically downward removes cleaning liquid carried from the bath by the wires. An enlarged jet is shown in Figure 3. The amount of liquid carried from a bath by a small wire is extremely great and losses because of this would be sufficient to render the process unduly expensive, if the liquid were permitted to be lost. In conventional plating baths the liquid is removed by wipes of cloth or other material, but in the present system such methods cannot be employed because of the tension necessarily imposed. The air blast satisfactorily removes the liquid from small wires and the wires feel dry to the touch after passing through the air. Similar air jets are provided after each bath. A single jet will take care of all of the wires under normal circumstances. In each case the jet is within the area bounded by the sump below the bath. Each bath, except the cold water washes, is provided with a sump 17, which need not be further described.

The wires pass from the first air jet 16 to the cold water rinse, thence under another air jet 16 into the acid pickle 4. This acid is preferably hydrochloric which is ordinary commercial hydrochloric diluted with from 1 to 4 parts of water. Overflow acid is recirculated by the pump 11a. The edges of this tank, as is the case with all of the other tanks, should have substantially the same level so that the overflows in all cases are within the catenary formed by the wire 25. The wires, after cleansing and neutralization in this bath, pass under another air jet 16 and into the water wash 5, into another jet 16 and into the plating bath 6.

For tin plating a fluoride tin bath of conventional composition may be employed. A suitable amperage is 500 per square foot but this may be varied to as low as 20 or as high as 1800. The amount of plating required for use in electric wiring is not great, generally being about 0.00002

inch. At 500 ft. per minute, and 500 amperes per square foot, the wire will acquire this coating in 9 feet of travel. The preferred bath has about this length.

5 A comb 30 may be provided at the entrance to the plating bath to spread the wires slightly. A similar comb may be supplied at the end of the bath. Normally, however, plating may be accomplished without the combs, and even where a comb is desirable, a single comb within the bath is usually sufficient.

As shown in the drawing, the bottom 15 of the bath, which is of metal and serves as the electrode, is sloped downwardly from the center in each 15 direction. The amount of this slope is such as to equalize the voltage drop through the solution. It must of course be varied with variations in the size of the wire and, for that reason, is preferably hinged at 15a to permit adjustment.

20 The plating fluid is heated in the sump by steam coils 9a preferably to a temperature in the neighborhood of 140° F. The liquid is circulated by a pump 11b and reintroduced at the bottom of the tank 6.

25 The wires pass from the plating bath under another air jet 16 through the overflow of the cold water wash 7, under another air jet 16 through the overflow of the hot water wash 8, under another air jet 16 and to the capstan 10. 30 The hot water wash is maintained at a temperature around 190° F. by steam coils 9 in the sump. Overflow is circulated to the bottom of the tank by the pump 11c. This hot water bath serves to assist the final air jet 16 by heating the wire 35 to a point where any remnant or trace of water is evaporated.

The capstan 10 is of conventional tapered shape and is so spaced that its take-up level is substantially the same as the level produced by the tensioning and spacing devices 22. The capstan is driven by a motor at a predetermined speed and the wire then passes to the spool 23 which is driven in conventional manner by a slipping belt under constant tension so that there is no slack in the wire or any superimposed tension beyond the desired amount.

It will be observed that the wires 25 are suspended in a catenary of small depth, which catenary is constantly changing as the wire advances and which maintains its shape. The catenary passes through the overflow of each of the baths, all of its contact with the liquids being confined to a layer of liquid having the depth of the catenary. As already stated, it is preferred to use a catenary having a depth of approximately  $\frac{1}{4}$  inch even over a space of approximately 30 feet.

55 Make-up water is supplied to the cold water tanks in any suitable fashion, as from overhead pipe 18.

The product produced by the herein described method is characterized by the fact that all of the plated metal occupies the same position with respect to underlying metal and to the center of the wire which it occupied at the time it was deposited. If it were attempted to electroplate wires of the type here described by ordinary methods, the wire would stretch as much as 40-50% of its length so that deposited metal would be displaced longitudinally and vertically with respect to its initially occupied position.

The foregoing detailed description has been given for clearness of understanding only, and no unnecessary limitations should be understood therefrom.

What I claim as new, and desire to secure by Letters Patent, is:

1. The method of simultaneously beaming and electroplating a plurality of wires of low elastic limit and small diameter which comprises passing a plurality of separate wires from separate let-off devices simultaneously through a series of baths including a plating bath, passing an electric current through the wires whereby a thin layer of plated metal is deposited thereon from the plating bath, the wires being under a common tension during plating but being laterally spaced in the plating bath and the wires being suspended throughout substantially their entire course in a catenary of small depth in which the wires form a single body wherein the wires are close together throughout substantially all of said catenary except within the plating bath, and then beaming the wires upon a take-up device connected by the wires to the let-off devices.

2. The method as set forth in claim 1 in which the entrance of the wires to and the exit of the

wires from each bath is through an overflow thereof.

ROBERT C. PIERCE.

#### REFERENCES CITED

The following references are of record in the file of this patent:

#### UNITED STATES PATENTS

|    | Number    | Name         | Date           |
|----|-----------|--------------|----------------|
| 10 | 242,813   | Chinnock     | June 14, 1881  |
|    | 1,068,412 | Chubb et al. | July 29, 1913  |
|    | 1,698,512 | Robbins      | Jan. 8, 1929   |
|    | 2,089,817 | Stutsman     | Aug. 10, 1937  |
| 15 | 2,093,238 | Domm         | Sept. 14, 1937 |

#### FOREIGN PATENTS

|    | Number  | Country       | Date          |
|----|---------|---------------|---------------|
| 20 | 19,586  | Great Britain | 1890          |
|    | 308,649 | Great Britain | June 25, 1930 |
|    | 495,907 | Great Britain | Nov. 21, 1930 |